



US009816163B2

(12) **United States Patent**  
**Douthett et al.**

(10) **Patent No.:** **US 9,816,163 B2**  
(45) **Date of Patent:** **Nov. 14, 2017**

(54) **COST-EFFECTIVE FERRITIC STAINLESS STEEL**

(2013.01); **C22C 38/44** (2013.01); **C22C 38/48** (2013.01); **C22C 38/50** (2013.01)

(71) Applicants: **Joseph A. Douthett**, Monroe, OH (US); **Shannon K. Craycraft**, Middletown, OH (US)

(58) **Field of Classification Search**

CPC ..... C22C 38/18-38/50  
USPC ..... 148/325; 420/61  
See application file for complete search history.

(72) Inventors: **Joseph A. Douthett**, Monroe, OH (US); **Shannon K. Craycraft**, Middletown, OH (US)

(56) **References Cited**

U.S. PATENT DOCUMENTS

|             |        |                   |
|-------------|--------|-------------------|
| 2,447,897 A | 8/1948 | Clarke, Jr.       |
| 2,797,993 A | 7/1957 | Tanczyn           |
| 3,833,359 A | 9/1974 | Murakami et al.   |
| 4,154,602 A | 5/1979 | Kaito et al.      |
| 4,690,798 A | 9/1987 | Narutani et al.   |
| 5,217,544 A | 6/1993 | Baltenneck et al. |
| 5,230,752 A | 7/1993 | Bourgain et al.   |

(Continued)

(73) Assignee: **AK Steel Properties, Inc.**

(\*) Notice: Subject to any disclaimer, the term of this patent is extended or adjusted under 35 U.S.C. 154(b) by 107 days.

(21) Appl. No.: **13/855,439**

(22) Filed: **Apr. 2, 2013**

FOREIGN PATENT DOCUMENTS

(65) **Prior Publication Data**

US 2013/0294960 A1 Nov. 7, 2013

|    |            |         |
|----|------------|---------|
| CA | 2707518 A1 | 7/2009  |
| CA | 2762899 A1 | 12/2010 |

(Continued)

**Related U.S. Application Data**

(60) Provisional application No. 61/619,048, filed on Apr. 2, 2012.

OTHER PUBLICATIONS

(51) **Int. Cl.**

|                   |           |
|-------------------|-----------|
| <b>C22C 38/20</b> | (2006.01) |
| <b>C22C 38/42</b> | (2006.01) |
| <b>C22C 38/44</b> | (2006.01) |
| <b>C22C 38/50</b> | (2006.01) |
| <b>C22C 38/00</b> | (2006.01) |
| <b>C22C 38/02</b> | (2006.01) |
| <b>C22C 38/04</b> | (2006.01) |
| <b>C22C 38/48</b> | (2006.01) |
| <b>C21D 6/00</b>  | (2006.01) |

(52) **U.S. Cl.**

|           |                                                                                                                                                                               |
|-----------|-------------------------------------------------------------------------------------------------------------------------------------------------------------------------------|
| CPC ..... | <b>C22C 38/001</b> (2013.01); <b>C21D 6/002</b> (2013.01); <b>C22C 38/02</b> (2013.01); <b>C22C 38/04</b> (2013.01); <b>C22C 38/20</b> (2013.01); <b>C22C 38/42</b> (2013.01) |
|-----------|-------------------------------------------------------------------------------------------------------------------------------------------------------------------------------|

(Continued)

*Primary Examiner* — Brian Walck

(74) *Attorney, Agent, or Firm* — Frost Brown Todd LLC

**ABSTRACT**

A cost effective ferritic stainless steel exhibits improved corrosion resistance comparable to that observed on Type 304L steel. The ferritic stainless steel is substantially nickel-free, dual stabilized with titanium and columbium, and contains chromium, copper, and molybdenum.

**16 Claims, 10 Drawing Sheets**



| References Cited         |         |                   |                 |
|--------------------------|---------|-------------------|-----------------|
| U.S. PATENT DOCUMENTS    |         |                   |                 |
| 5,304,259 A              | 4/1994  | Miyakusu et al.   | 8,062,584 B2    |
| 5,395,583 A              | 3/1995  | Potgieter et al.  | 8,152,937 B2    |
| 5,427,635 A              | 6/1995  | Bleton et al.     | 8,153,055 B2    |
| 5,492,575 A              | 2/1996  | Teraoka et al.    | 8,226,780 B2    |
| 5,565,167 A              | 10/1996 | Fujimoto et al.   | 8,268,101 B2    |
| 5,656,237 A              | 8/1997  | Terrien et al.    | 8,287,805 B2    |
| 5,714,115 A              | 2/1998  | Speidel et al.    | 8,303,733 B2    |
| 5,773,734 A              | 6/1998  | Young             | 8,333,849 B2    |
| 5,779,820 A              | 7/1998  | Hauser et al.     | 8,333,851 B2    |
| 5,785,924 A              | 7/1998  | Beguinot et al.   | 8,337,748 B2    |
| 5,795,411 A              | 8/1998  | Terrien et al.    | 8,337,749 B2    |
| 5,830,408 A              | 11/1998 | Azuma et al.      | 8,357,247 B2    |
| 5,868,875 A              | 2/1999  | Yoshitake et al.  | 8,506,727 B2    |
| 6,033,625 A              | 3/2000  | Nagashima et al.  | 8,535,606 B2    |
| 6,048,416 A              | 4/2000  | Hauser et al.     | 8,540,933 B2    |
| 6,056,917 A              | 5/2000  | Chesseret et al.  | 8,562,758 B2    |
| 6,086,689 A              | 7/2000  | Sassoulas et al.  | 8,580,048 B2    |
| 6,096,441 A              | 8/2000  | Hauser et al.     | 8,608,873 B2    |
| 6,106,639 A              | 8/2000  | Marandet et al.   | 8,663,549 B2    |
| 6,110,300 A              | 8/2000  | Brada et al.      | 8,721,960 B2    |
| 6,123,784 A              | 9/2000  | Havette           | 8,790,573 B2    |
| 6,159,310 A              | 12/2000 | Inoue et al.      | 8,877,121 B2    |
| 6,168,756 B1             | 1/2001  | Hirasawa et al.   | 8,894,924 B2    |
| 6,171,547 B1             | 1/2001  | Sagara et al.     | 8,980,167 B2    |
| 6,235,237 B1             | 5/2001  | Osing et al.      | 9,150,947 B2    |
| 6,294,131 B1             | 9/2001  | Jaffrey           | 9,181,824 B2    |
| 6,352,670 B1             | 3/2002  | Rakowski          | 9,279,172 B2    |
| 6,379,476 B1             | 4/2002  | Tarutani et al.   | 9,290,845 B2    |
| 6,409,847 B2             | 6/2002  | Kleemann          | 2002/0033210 A1 |
| 6,423,159 B1             | 7/2002  | Liesert et al.    | 2003/0086810 A1 |
| 6,426,039 B2             | 7/2002  | Hirasawa et al.   | 2003/0172999 A1 |
| 6,440,236 B1             | 8/2002  | Hiramatsu et al.  | 2004/0040631 A1 |
| 6,440,579 B1             | 8/2002  | Hauser et al.     | 2004/0050462 A1 |
| 6,485,680 B2             | 11/2002 | Ragot et al.      | 2004/0074574 A1 |
| 6,500,280 B2             | 12/2002 | Ota et al.        | 2004/0156737 A1 |
| 6,521,056 B2             | 2/2003  | Muraki et al.     | 2004/0166015 A1 |
| 6,547,891 B2             | 4/2003  | Linden et al.     | 2004/0244884 A1 |
| 6,551,420 B1             | 4/2003  | Bergstrom et al.  | 2005/0139298 A1 |
| 6,564,990 B2             | 5/2003  | Nagashima et al.  | 2005/0217769 A1 |
| 6,582,835 B2             | 6/2003  | Antoni et al.     | 2005/0269074 A1 |
| 6,592,685 B2             | 7/2003  | Goecmen           | 2006/0008694 A1 |
| 6,623,569 B2             | 9/2003  | Bergstrom et al.  | 2006/0150388 A1 |
| 6,645,324 B2             | 11/2003 | Hirata et al.     | 2006/0266439 A1 |
| 6,673,165 B2             | 1/2004  | Koga et al.       | 2006/0285989 A1 |
| 6,673,166 B2             | 1/2004  | Oku et al.        | 2007/0089810 A1 |
| 6,682,582 B1             | 1/2004  | Speidel           | 2007/0187002 A1 |
| 6,682,780 B2             | 1/2004  | Tzatzov et al.    | 2008/0073004 A1 |
| 6,692,592 B2             | 2/2004  | Kidani et al.     | 2008/0206088 A1 |
| 6,696,016 B1             | 2/2004  | Kimura            | 2009/0032246 A1 |
| 6,723,181 B2             | 4/2004  | Ishikawa et al.   | 2009/0053093 A1 |
| 6,740,174 B2             | 5/2004  | Miyazaki et al.   | 2009/0060775 A1 |
| 6,793,744 B1             | 9/2004  | Jung              | 2009/0111607 A1 |
| 6,793,746 B2             | 9/2004  | Shimizu et al.    | 2009/0324441 A1 |
| 6,855,213 B2             | 2/2005  | Yoshitake et al.  | 2010/0000636 A1 |
| 6,921,440 B2             | 7/2005  | Liesert et al.    | 2010/0133096 A1 |
| 7,081,173 B2             | 7/2006  | Bahar et al.      | 2010/0183475 A1 |
| 7,094,295 B2             | 8/2006  | Oku et al.        | 2010/0189589 A1 |
| 7,166,174 B2             | 1/2007  | De Bondt et al.   | 2010/0223927 A1 |
| 7,255,755 B2             | 8/2007  | Maziasz et al.    | 2010/0272593 A1 |
| 7,335,428 B2             | 2/2008  | Fraisse et al.    | 2011/0061777 A1 |
| 7,341,690 B2             | 3/2008  | Miyazaki et al.   | CA 2860746 A1   |
| 7,343,730 B2             | 3/2008  | Humcke et al.     | CN 86101805 A   |
| 7,476,282 B2             | 1/2009  | Tanida et al.     | CN 101680066 A  |
| 7,531,129 B2             | 5/2009  | Igarashi et al.   | CN 101784686 A  |
| 7,572,407 B2             | 8/2009  | Hirasawa et al.   | EP 0547626      |
| 7,731,895 B2             | 6/2010  | Okada et al.      | EP 0638653      |
| 7,749,431 B2             | 7/2010  | Igarashi et al.   | JP S56-146857 A |
| RE41,504 E               | 8/2010  | Maziasz et al.    | JP S58-39732 A  |
| 7,767,037 B2             | 8/2010  | Kimura et al.     | JP S60-2622 A   |
| 7,780,798 B2             | 8/2010  | Stinson et al.    | JP H04-280948 A |
| 7,819,991 B2             | 10/2010 | Kato et al.       | JP H08-199314 A |
| 7,842,141 B2             | 11/2010 | Kimura et al.     | JP H08 246105   |
| 7,923,126 B2             | 4/2011  | Gudme             | JP H08 311543   |
| 7,981,561 B2             | 7/2011  | Rakowski et al.   | JP H09 227999   |
| 8,025,839 B2             | 9/2011  | Jonson et al.     | JP H09 228002   |
|                          |         |                   | JP H10 81940    |
| FOREIGN PATENT DOCUMENTS |         |                   |                 |
| 8,152,937 B2             | 4/2012  | Ishii et al.      | 8/1986          |
| 8,153,055 B2             | 4/2012  | Nakamura et al.   | 3/2010          |
| 8,226,780 B2             | 7/2012  | Hatano et al.     | 7/2010          |
| 8,268,101 B2             | 9/2012  | Conrad et al.     | 6/1993          |
| 8,287,805 B2             | 10/2012 | Sjodin            | 2/1995          |
| 8,303,733 B2             | 11/2012 | Hamada et al.     | 3/2015          |
| 8,333,849 B2             | 12/2012 | Yamauchi et al.   | 9/1997          |
| 8,333,851 B2             | 12/2012 | Suwabe            | 9/2013          |
| 8,337,748 B2             | 12/2012 | Rakowski et al.   | 3/2016          |
| 8,337,749 B2             | 12/2012 | Bergstrom et al.  | 10/2013         |
| 8,357,247 B2             | 1/2013  | Hirasawa et al.   | 5/2014          |
| 8,506,727 B2             | 8/2013  | Pelsoeczy         | 10/2015         |
| 8,535,606 B2             | 9/2013  | John              | 11/2015         |
| 8,540,933 B2             | 9/2013  | Nylof et al.      | 12/2014         |
| 8,562,758 B2             | 10/2013 | Fujisawa et al.   | 1/2014          |
| 8,580,048 B2             | 11/2013 | Pelsoeczy         | 2/2015          |
| 8,608,873 B2             | 12/2013 | Abbatis et al.    | 3/2016          |
| 8,663,549 B2             | 3/2014  | Ohishi et al.     | 4/2014          |
| 8,721,960 B2             | 5/2014  | Hatano et al.     | 5/2015          |
| 8,790,573 B2             | 7/2014  | Miyazaki et al.   | 6/2015          |
| 8,877,121 B2             | 11/2014 | Bergstrom et al.  | 7/2015          |
| 8,894,924 B2             | 11/2014 | Matsuhashi et al. | 8/2015          |
| 8,980,167 B2             | 3/2015  | Kimura et al.     | 9/2015          |
| 9,150,947 B2             | 10/2015 | Nishiyama et al.  | 10/2015         |
| 9,181,824 B2             | 11/2015 | Montagnon         | 11/2015         |
| 9,279,172 B2             | 3/2016  | Kato et al.       | 12/2015         |
| 9,290,845 B2             | 3/2016  | Kim et al.        | 1/2016          |
| 2002/0033210 A1          | 3/2002  | Fujitsuna et al.  | 2/2002          |
| 2003/0086810 A1          | 5/2003  | Schnabel et al.   | 3/2003          |
| 2003/0172999 A1          | 9/2003  | Alfonsson et al.  | 4/2003          |
| 2004/0040631 A1          | 3/2004  | Takahashi et al.  | 5/2004          |
| 2004/0050462 A1          | 3/2004  | Grubb             | 6/2004          |
| 2004/0074574 A1          | 4/2004  | Kimura            | 7/2004          |
| 2004/0156737 A1          | 8/2004  | Rakowski          | 8/2004          |
| 2004/0166015 A1          | 8/2004  | Kimura            | 9/2004          |
| 2004/0244884 A1          | 12/2004 | Hidemitsu et al.  | 10/2004         |
| 2005/0139298 A1          | 6/2005  | Pacher et al.     | 7/2005          |
| 2005/0217769 A1          | 10/2005 | Pacher et al.     | 8/2005          |
| 2005/0269074 A1          | 12/2005 | Chitwood          | 9/2005          |
| 2006/0008694 A1          | 1/2006  | Budinski et al.   | 10/2006         |
| 2006/0150388 A1          | 7/2006  | Inada et al.      | 11/2006         |
| 2006/0266439 A1          | 11/2006 | Maziasz et al.    | 12/2006         |
| 2006/0285989 A1          | 12/2006 | Schade            | 1/2007          |
| 2007/0089810 A1          | 4/2007  | Sundstrom et al.  | 2/2007          |
| 2007/0187002 A1          | 8/2007  | Takahashi et al.  | 3/2007          |
| 2008/0073004 A1          | 3/2008  | Pacher et al.     | 4/2008          |
| 2008/0206088 A1          | 8/2008  | Cusolito et al.   | 9/2008          |
| 2009/0032246 A1          | 2/2009  | Takabe et al.     | 3/2009          |
| 2009/0053093 A1          | 2/2009  | Oku et al.        | 4/2009          |
| 2009/0060775 A1          | 3/2009  | Liu               | 5/2009          |
| 2009/0111607 A1          | 4/2009  | Taylor et al.     | 6/2009          |
| 2009/0324441 A1          | 12/2009 | Weiss et al.      | 1/2010          |
| 2010/0000636 A1          | 1/2010  | Bonnefois et al.  | 2/2010          |
| 2010/0133096 A1          | 6/2010  | Hansen et al.     | 3/2010          |
| 2010/0183475 A1          | 7/2010  | Radon et al.      | 4/2010          |
| 2010/0189589 A1          | 7/2010  | Liu               | 5/2010          |
| 2010/0223927 A1          | 9/2010  | Oku et al.        | 6/2010          |
| 2010/0272593 A1          | 10/2010 | Ishikawa et al.   | 7/2010          |
| 2011/0061777 A1          | 3/2011  | Ishii et al.      | 8/2011          |

(56)

**References Cited**

## FOREIGN PATENT DOCUMENTS

JP 2006-097908 A 4/2006  
JP 2006-131945 5/2006  
JP 2006-257544 A 9/2006  
JP 2007-131870 A 5/2007  
JP 2007-302995 A 11/2007  
JP 2008-291303 A 12/2008  
JP 2009-035813 A 2/2009  
JP 2010-202916 A 9/2010  
JP 2010-202973 A 9/2010  
JP 2011-179116 9/2011  
RU 2132886 C1 7/1999  
RU 2242325 C2 12/2004  
RU 2429306 C1 9/2011  
TW I482866 B 5/2015  
UA 111115 C2 3/2016  
WO WO 2008/156195 A1 12/2008

## OTHER PUBLICATIONS

International Search Report and Written Opinion dated Jul. 24, 2013 for Application No. PCT/US2013/034940.  
English Abstract of Japanese Patent No. JP H08 246105.  
English Abstract of Japanese Patent No. JP H08 311543.  
English Abstract of Japanese Patent No. JP H09 227999.  
English Abstract of Japanese Patent No. JP H09 228002.  
English Abstract of Japanese Patent No. JP H10 91940.  
“JFE443CT, Ni, Mo-free stainless steel with high corrosion resistance: 21Cr Stainless Steel,” JFE Steel Corporation, Catalog No. G1E-004-03, 2012, accessed from: <http://www.jfe-steel.co.jp/en/products/stainless/catalog/gle-004.pdf>.

Canadian Office Action dated Jan. 22, 2016 for Application No. CA 2,868,278, 6 pgs.

Chinese Office Action dated Sep. 18, 2015 for Application No. CN 201380018563.7, 8 pgs.

European Exam Report dated Sep. 1, 2015 for Application No. EP 13716682.3, 5 pgs.

Japanese Office Action dated Nov. 10, 2015 for Application No. JP 2015-504675, 9 pgs.

Korean Office Action dated Oct. 12, 2015 for Application No. KR 10-2014-7030826, 5 pgs.

Russian Office Action dated Apr. 8, 2016 for Application No. RU 2014138182/02(061887), 14 pgs.

Taiwanese Search Report dated Jun. 23, 2014 for Application No. TW 102111957, 6 pgs.

Ukrainian Office Action dated Dec. 12, 2014 for Application No. UA a 2014 10374, 4 pgs.

Korean Office Action, Notice of Final Rejection, dated Feb. 16, 2017 for Application No. 10-2014-7030826, 6 pages.

Australian Office Action dated Oct. 6, 2016 for Application No. 2013243635, 3 pages.

Canadian Office Action dated Nov. 23, 2016 for Application No. 2,868,278, 3 pages.

Chinese Office Action dated May 10, 2016 for Application No. 201380018563.7, 8 pages.

Chinese Office Action dated Dec. 8, 2016 for Application No. 201380018563.7, 11 pages.

Japanese Office Action, Examiner's Decision of Refusal, dated Aug. 16, 2016 for Application No. 2015-504675, 8 pages.

Korean Office Action, Notice of Final Rejection, dated Jun. 20, 2016 for Application No. 10-2014-7030826, 6 pages.

Korean Office Action, Notice of Preliminary Rejection, dated Sep. 27, 2016 for Application No. 10-2014-7030826, 7 pages.

Russian Office Action, Notice of Allowance, dated Jul. 8, 2016 for Application No. 2014138182/02, 13 pages.

Figure 1



Figure 2



Figure 3



Figure 4



Figure 5



Figure 6



Figure 7



Figure 8



Figure 9



Figure 10

## Potentiodynamic Behavior of ID 92 in 3.5% Sodium Chloride



## 1

## COST-EFFECTIVE FERRITIC STAINLESS STEEL

This application is a non-provisional patent application claiming priority from provisional application Ser. No. 61/619,048 entitled "21% Cr Ferritic Stainless Steel," filed on Apr. 2, 2012. The disclosure of application Ser. No. 61/619,048 is incorporated herein by reference.

## SUMMARY

It is desirable to produce a ferritic stainless steel with corrosion resistance comparable to that of ASTM Type 304 stainless steel but that is substantially nickel-free, dual stabilized with titanium and columbium to provide protection from intergranular corrosion, and contains chromium, copper, and molybdenum to provide pitting resistance without sacrificing stress corrosion cracking resistance. Such a steel is particularly useful for commodity steel sheet commonly found in commercial kitchen applications, architectural components, and automotive applications, including but not limited to commercial and passenger vehicle exhaust and selective catalytic reduction (SCR) components.

## BRIEF DESCRIPTION OF THE DRAWINGS

FIG. 1 is a phase diagram for elements of titanium and nitrogen at the liquidus temperature for an embodiment of the ferritic stainless steel.

FIG. 2 is a graph depicting corrosion rate as a function of steel composition in a reducing acidic chloride environment such as hydrochloric acid.

FIG. 3 is a graph depicting corrosion rate as a function of steel composition in a reducing acid that is sulfate rich.

FIG. 4 is a graph depicting electrochemical anodic dissolution current density as a function of steel composition.

FIG. 5 is a graph depicting electrochemical breakdown potential as a function of steel composition.

FIG. 6 is a graph depicting electrochemical breakdown potential as a function of steel composition.

FIG. 7 is a graph depicting electrochemical repassivation potential as a function of steel composition.

FIG. 8 is a graph depicting electrochemical repassivation potential as a function of steel composition.

FIG. 9 is a graph depicting comparative potentiostatic behavior of a ferritic stainless steel and a comparative steel.

FIG. 10 graph depicting comparative potentiodynamic behavior of a ferritic stainless steel and a comparative steel.

## DETAILED DESCRIPTION

In the ferritic stainless steels, the inter-relationship of and amount of titanium, columbium, carbon, and nitrogen are controlled to achieve subequilibrium surface quality, substantially equiaxed cast grain structure, and substantially full stabilization against intergranular corrosion. In addition, the inter-relationship of chromium, copper, and molybdenum is controlled to optimize corrosion resistance.

Subequilibrium melts are typically defined as compositions with titanium and nitrogen levels low enough so that they do not form titanium nitrides in the alloy melt. Such precipitates can form defects, such as surface stringer defects or laminations, during hot or cold rolling. Such defects can diminish formability, corrosion resistance, and appearance. FIG. 1 was derived from an exemplary phase diagram, created using thermodynamic modeling for elements of titanium and nitrogen at the liquidus temperature

## 2

for an embodiment of the ferritic stainless steel. To be substantially free of titanium nitrides and be considered subequilibrium, the titanium and nitrogen levels in the ferritic stainless steel should fall to the left or lower portion of the solubility curve shown in FIG. 1. The titanium nitride solubility curve, as shown in FIG. 1, can be represented mathematically as follows:

$$Ti_{max} = 0.0044(N^{-1.027})$$

Equation 1:

10 where  $Ti_{max}$  is the maximum concentration of titanium by percent weight, and N is the concentration of nitrogen by percent weight. All concentrations herein will be reported by percent weight, unless expressly noted otherwise.

Using Equation 1, if the nitrogen level is maintained at or 15 below 0.020% in an embodiment, then the titanium concentration for that embodiment should be maintained at or below 0.25%. Allowing the titanium concentration to exceed 0.25% can lead to the formation of titanium nitride precipitates in the molten alloy. However, FIG. 1 also shows that 20 titanium levels above 0.25% can be tolerated if the nitrogen levels are less than 0.02%.

Embodiments of the ferritic stainless steels exhibit an equiaxed cast and rolled and annealed grain structure with no large columnar grains in the slabs or banded grains in the 25 rolled sheet. This refined grain structure can improve formability and toughness. To achieve this grain structure, there should be sufficient titanium, nitrogen and oxygen levels to seed the solidifying slabs and provide sites for equiaxed grains to initiate. In such embodiments, the minimum titanium and nitrogen levels are shown in FIG. 1, and expressed 30 by the following equation:

$$Ti_{min} = 0.0025/N$$

Equation 2:

where  $Ti_{min}$  is the minimum concentration of titanium by 35 percent weight, and N is the concentration of nitrogen by percent weight.

Using the Equation 2, if the nitrogen level is maintained at or below 0.02% in an embodiment, the minimum titanium concentration is 0.125%. The parabolic curve depicted in 40 FIG. 1 reveals an equiaxed grain structure can be achieved at nitrogen levels above 0.02% nitrogen if the total titanium concentration is reduced. An equiaxed grain structure is expected with titanium and nitrogen levels to the right or above of plotted Equation 2. This relationship between 45 subequilibrium and titanium and nitrogen levels that produced equiaxed grain structure is illustrated in FIG. 1, in which the minimum titanium equation (Equation 2) is plotted on the liquidus phase diagram of FIG. 1. The area between the two parabolic lines is the range of titanium and nitrogen levels in the embodiments.

Fully stabilized melts of the ferritic stainless steels must have sufficient titanium and columbium to combine with the 50 soluble carbon and nitrogen present in the steel. This helps to prevent chromium carbide and nitrides from forming and 55 lowering the intergranular corrosion resistance. The minimum titanium and carbon necessary to lead to full stabilization is best represented by the following equation:

$$Ti + Cb_{min} = 0.2\% + 4(C + N)$$

Equation 3:

60 where Ti is the amount of titanium by percent weight,  $Cb_{min}$  is the minimum amount of columbium by percent weight, C is the amount of carbon by percent weight, and N is the amount of nitrogen by percent weight.

In the embodiments described above, the titanium level 65 necessary for an equiaxed grain structure and subequilibrium conditions was determined when the maximum nitrogen level was 0.02%. As explained above, the respective

Equations 1 and 2 yielded 0.125% minimum titanium and 0.25% maximum titanium. In such embodiments, using a maximum of 0.025% carbon and applying Equation 3, would require minimum columbium contents of 0.25% and 0.13%, respectively for the minimum and maximum titanium levels. In some such embodiments, the aim for the concentration of columbium would be 0.25%.

In certain embodiments, keeping the copper level between 0.40-0.80% in a matrix consisting of about 21% Cr and 0.25% Mo one can achieve an overall corrosion resistance that is comparable if not improved to that found in commercially available Type 304L. The one exception may be in the presence of a strongly acidic reducing chloride like hydrochloric acid. The copper-added alloys show improved performance in sulfuric acid. When the copper level is maintained between 0.4-0.8%, the anodic dissolution rate is reduced and the electrochemical breakdown potential is maximized in neutral chloride environments. In some embodiments, the optimal Cr, Mo, and Cu level, in weight percent satisfies the following two equations:

$$20.5 \leq \text{Cr} + 3.3\text{Mo}$$

Equation 4:

$$0.6 \leq \text{Cu} + \text{Mo} \leq 1.4 \text{ when } \text{Cu}_{max} < 0.80$$

Equation 5:

Embodiments of the ferritic stainless steel can contain carbon in amounts of about 0.020 or less percent by weight.

Embodiments of the ferritic stainless steel can contain manganese in amounts of about 0.40 or less percent by weight.

Embodiments of the ferritic stainless steel can contain phosphorus in amounts of about 0.030 or less percent by weight.

Embodiments of the ferritic stainless steel can contain sulfur in amounts of about 0.010 or less percent by weight.

Embodiments of the ferritic stainless steel can contain silicon in amounts of about 0.30-0.50 percent by weight. Some embodiments can contain about 0.40% silicon.

Embodiments of the ferritic stainless steel can contain chromium in amounts of about 20.0-23.0 percent by weight. Some embodiments can contain about 21.5-22 percent by weight chromium, and some embodiments can contain about 21.75% chromium.

Embodiments of the ferritic stainless steel can contain nickel in amounts of about 0.40 or less percent by weight.

Embodiments of the ferritic stainless steel can contain nitrogen in amounts of about 0.020 or less percent by weight.

Embodiments of the ferritic stainless steel can contain copper in amounts of about 0.40-0.80 percent by weight. Some embodiments can contain about 0.45-0.75 percent by weight copper and some embodiments can contain about 0.60% copper.

Embodiments of the ferritic stainless steel can contain molybdenum in amounts of about 0.20-0.60 percent by weight. Some embodiments can contain about 0.30-0.5 percent by weight molybdenum, and some embodiments can contain about 0.40% molybdenum.

Embodiments of the ferritic stainless steel can contain titanium in amounts of about 0.10-0.25 percent by weight. Some embodiments can contain about 0.17-0.25 percent by weight titanium, and some embodiments can contain about 0.21% titanium.

Embodiments of the ferritic stainless steel can contain columbium in amounts of about 0.20-0.30 percent by weight. Some embodiments can contain about 0.25% columbium.

Embodiments of the ferritic stainless steel can contain aluminum in amounts of about 0.010 or less percent by weight.

The ferritic stainless steels are produced using process conditions known in the art for use in manufacturing ferritic stainless steels, such as the processes described in U.S. Pat. Nos. 6,855,213 and 5,868,875.

In some embodiments, the ferritic stainless steels may also include other elements known in the art of steelmaking that can be made either as deliberate additions or present as residual elements, i.e., impurities from steelmaking process.

A ferrous melt for the ferritic stainless steel is provided in a melting furnace such as an electric arc furnace. This ferrous melt may be formed in the melting furnace from solid iron bearing scrap, carbon steel scrap, stainless steel scrap, solid iron containing materials including iron oxides, iron carbide, direct reduced iron, hot briquetted iron, or the melt may be produced upstream of the melting furnace in a blast furnace or any other iron smelting unit capable of providing a ferrous melt. The ferrous melt then will be refined in the melting furnace or transferred to a refining vessel such as an argon-oxygen-decarburization vessel or a vacuum-oxygen-decarburization vessel, followed by a trim station such as a ladle metallurgy furnace or a wire feed station.

In some embodiments, the steel is cast from a melt containing sufficient titanium and nitrogen but a controlled amount of aluminum for forming small titanium oxide inclusions to provide the necessary nuclei for forming the as-cast equiaxed grain structure so that an annealed sheet produced from this steel also has enhanced ridging characteristics.

In some embodiments, titanium is added to the melt for deoxidation prior to casting. Deoxidation of the melt with titanium forms small titanium oxide inclusions that provide the nuclei that result in an as-cast equiaxed fine grain structure. To minimize formation of alumina inclusions, i.e., aluminum oxide,  $\text{Al}_2\text{O}_3$ , aluminum may not be added to this refined melt as a deoxidant. In some embodiments, titanium and nitrogen can be present in the melt prior to casting so that the ratio of the product of titanium and nitrogen divided by residual aluminum is at least about 0.14.

If the steel is to be stabilized, sufficient amount of the titanium beyond that required for deoxidation can be added for combining with carbon and nitrogen in the melt but preferably less than that required for saturation with nitrogen, i.e., in a sub-equilibrium amount, thereby avoiding or at least minimizing precipitation of large titanium nitride inclusions before solidification.

The cast steel is hot processed into a sheet. For this disclosure, the term "sheet" is meant to include continuous strip or cut lengths formed from continuous strip and the term "hot processed" means the as-cast steel will be reheated, if necessary, and then reduced to a predetermined thickness such as by hot rolling. If hot rolled, a steel slab is reheated to 2000° to 2350° F. (1093°-1288° C.), hot rolled using a finishing temperature of 1500-1800° F. (816-982° C.) and coiled at a temperature of 1000-1400° F. (538-760° C.). The hot rolled sheet is also known as the "hot band." In some embodiments, the hot band may be annealed at a peak metal temperature of 1700-2100° F. (926-1149° C.). In some embodiments, the hot band may be descaled and cold reduced at least 40% to a desired final sheet thickness. In other embodiments, the hot band may be descaled and cold reduced at least 50% to a desired final sheet thickness. Thereafter, the cold reduced sheet can be final annealed at a peak metal temperature of 1700-2100° F. (927-1149° C.).

The ferritic stainless steel can be produced from a hot processed sheet made by a number of methods. The sheet can be produced from slabs formed from ingots or continuous cast slabs of 50-200 mm thickness which are reheated to 2000° to 2350° F. (1093°-1288° C.) followed by hot rolling to provide a starting hot processed sheet of 1-7 mm thickness or the sheet can be hot processed from strip continuously cast into thicknesses of 2-26 mm. The present process is applicable to sheet produced by methods wherein continuous cast slabs or slabs produced from ingots are fed directly to a hot rolling mill with or without significant reheating, or ingots hot reduced into slabs of sufficient temperature to be hot rolled in to sheet with or without further reheating.

#### EXAMPLE 1

To prepare ferritic stainless steel compositions that resulted in an overall corrosion resistance comparable to Type 304L austenitic stainless steel a series of laboratory heats were melted and analyzed for resistance to localized corrosion.

The first set of heats was laboratory melted using air melt capabilities. The goal of this series of air melts was to better understand the role of chromium, molybdenum, and copper in a ferritic matrix and how the variations in composition compare to the corrosion behavior of Type 304L steel. For this study the compositions of embodiments used in the air melts investigated are set forth in Table 1 as follows:

TABLE 1

| Code | Stencil | C     | Mn   | P     | S      | Si   | Cr    | Ni   | Cu   | Mo    | N     | Cb   | Ti   |
|------|---------|-------|------|-------|--------|------|-------|------|------|-------|-------|------|------|
| A    | 251     | 0.016 | 0.36 | 0.033 | 0.0016 | 0.4  | 20.36 | 0.25 | 0.5  | 0.002 | 0.024 | 0.2  | 0.15 |
| B    | 302     | 0.013 | 0.33 | 0.033 | 0.0015 | 0.39 | 20.36 | 0.25 | 0.48 | 0.25  | 0.024 | 0.2  | 0.11 |
| C    | 262     | 0.014 | 0.31 | 0.032 | 0.0015 | 0.37 | 20.28 | 0.25 | 0.48 | 0.49  | 0.032 | 0.19 | 0.13 |
| D    | 301     | 0.012 | 0.34 | 0.032 | 0.0017 | 0.39 | 20.37 | 0.25 | 0.09 | 0.25  | 0.024 | 0.2  | 0.15 |
| E    | 272     | 0.014 | 0.3  | 0.031 | 0.0016 | 0.36 | 20.22 | 0.24 | 1.01 | 0.28  | 0.026 | 0.19 | 0.12 |
| F    | 271     | 0.014 | 0.31 | 0.032 | 0.0015 | 0.36 | 18.85 | 0.25 | 0.49 | 0.28  | 0.024 | 0.2  | 0.15 |
| G    | 28      | 0.012 | 0.36 | 0.033 | 0.0016 | 0.41 | 21.66 | 0.25 | 0.49 | 0.25  | 0.026 | 0.2  | 0.12 |
| H    | 29      | 0.014 | 0.35 | 0.033 | 0.0014 | 0.41 | 20.24 | 0.25 | 1    | 0.5   | 0.026 | 0.18 | 0.15 |

Both ferric chloride immersion and electrochemical evaluations were performed on all the above mentioned chemistries in Table 1 and compared to the performance of Type 304L steel.

Following methods described in ASTM 648 Ferric Chloride Pitting Test Method A, specimens were evaluated for mass loss after a 24 hour exposure to 6% Ferric Chloride solution at 50° C. This test exposure evaluates the basic

tent of 1% did not perform as well as the other chemistries. However, this behavior may have been as a result of less than ideal surface quality due to the melting process.

A closer investigation of the passive film strength and repassivation behavior was studied using electrochemical techniques that included both corrosion behavior diagrams (CBD) and cycle polarization in a deaerated, dilute, neutral chloride environment. The electrochemical behavior observed on this set of air melts showed that a combination of approximately 21% Cr while in the presence of approximately 0.5% Cu and a small Mo addition achieved three primary improvements to Type 304L steel. First, the copper addition appeared to slow the initial anodic dissolution rate at the surface; second, the copper and small molybdenum presence in the 21% Cr chemistry assisted in a strong passive film formation; and third, the molybdenum and high chromium content assisted in the improved repassivation behavior. The level of copper in the 21Cr+ residual Mo melt chemistry did appear to have an "optimal" level in that adding 1% Cu resulted in diminished return. This confirms the behavior observed in the ferric chloride pitting test. Additional melt chemistries were submitted for vacuum melting in hopes to create cleaner steel specimens and

determine the optimal copper addition in order to achieve the best overall corrosion resistance.

#### EXAMPLE 2

The second set of melt chemistries set forth in Table 2 was submitted for vacuum melt process. The compositions in this study are shown below:

TABLE 2

| ID | C     | Mn   | P     | S      | Si   | Cr    | Ni   | Cu   | Mo   | N     | Cb   | Ti   |
|----|-------|------|-------|--------|------|-------|------|------|------|-------|------|------|
| 02 | 0.015 | 0.30 | 0.027 | 0.0026 | 0.36 | 20.82 | 0.25 | 0.24 | 0.25 | 0.014 | 0.20 | 0.15 |
| 51 | 0.014 | 0.30 | 0.026 | 0.0026 | 0.36 | 20.76 | 0.24 | 0.94 | 0.25 | 0.014 | 0.20 | 0.17 |
| 91 | 0.016 | 0.29 | 0.028 | 0.0026 | 0.35 | 20.72 | 0.25 | 0.48 | 0.25 | 0.014 | 0.20 | 0.17 |
| 92 | 0.016 | 0.29 | 0.028 | 0.0026 | 0.36 | 20.84 | 0.25 | 0.74 | 0.25 | 0.014 | 0.20 | 0.15 |

resistance to pitting corrosion while exposed to an acidic, strongly oxidizing, chloride environment.

The screening test suggested that higher chromium bearing ferritic alloys that have a small copper addition would result in the most corrosion resistance composition within the series. The composition having the highest copper con-

tent of 1% did not perform as well as the other chemistries. However, this behavior may have been as a result of less than ideal surface quality due to the melting process.

The above mentioned heats varied mainly in copper content. Additional vacuum heats, of the compositions set forth in Table 3, were also melted for comparison purposes. The Type 304L steel used for comparison was commercially available sheet.

TABLE 3

| ID   | C     | Mn   | P     | S      | Si   | Cr    | Ni   | Cu     | Mo     | N      | Cb   | Ti   |
|------|-------|------|-------|--------|------|-------|------|--------|--------|--------|------|------|
| 31   | 0.016 | 0.33 | 0.028 | 0.0030 | 0.42 | 20.70 | 0.24 | <0.002 | <0.002 | 0.0057 | 0.21 | 0.15 |
| 41   | 0.016 | 0.32 | 0.027 | 0.0023 | 0.36 | 18.63 | 0.25 | 0.48   | 0.24   | 0.014  | 0.18 | 0.16 |
| 52   | 0.015 | 0.30 | 0.026 | 0.0026 | 0.36 | 20.78 | 0.24 | 0.94   | 0.25   | 0.014  | 0.20 | 0.16 |
| 304L | 0.023 | 1.30 | 0.040 | 0.005  | 0.35 | 18.25 | 8.10 | —      | 0.50   | 0.030  | —    | —    |
| AIM  |       |      |       | max    |      |       |      |        | max    |        |      |      |

The chemistries of Table 3 were vacuum melted into ingots, hot rolled at 2250 F (1232° C.), descaled and cold reduced 60%. The cold reduced material had a final anneal at 1825 F (996° C.) followed by a final descale.

### EXAMPLE 3

Comparison studies performed on the above mentioned vacuum melts of Example 2 (identified by their ID numbers) were chemical immersion tested in hydrochloric acid, sulfuric acid, sodium hypochlorite, and acetic acid.

#### 1% Hydrochloric Acid.

As shown in FIG. 2, the chemical immersion evaluations showed the beneficial effects of nickel in a reducing acidic chloride environment such as hydrochloric acid. Type 304L steel outperformed all of the chemistries studied in this environment. The addition of chromium resulted in a lower overall corrosion rate and the presence of copper and molybdenum showed a further reduction of corrosion rate but the effects of copper alone were minimal as shown by the graph of the line identified as Fe21CrXCu0.25Mo in FIG. 2. This behavior supports the benefits of nickel additions for service conditions such as the one described below.

#### 5% Sulfuric Acid.

As shown in FIG. 3, in an immersion test consisting of a reducing acid that is sulfate rich, alloys with chromium levels between 18-21% behaved similarly. The addition of molybdenum and copper significantly reduced the overall corrosion rate. When evaluating the effects of copper alone on the corrosion rate (as indicated by the graph of the line identified as Fe21CrXCu0.25Mo in FIG. 3), it appeared as though there is a direct relationship in that the higher the copper, the lower the corrosion rate. At the 0.75% copper level the overall corrosion rate began to level off and was within 2 mm/yr of 304L steel. Molybdenum at the 0.25% level tends to play a large role in the corrosion rate in sulfuric acid. However, the dramatic reduction in rate was also attributed to the copper presence. Though the alloys of Example 2 did not have a rate of corrosion below Type 304L steel they did show improved and comparable corrosion resistance under reducing sulfuric acid conditions.

#### Acetic Acid and Sodium Hypochlorite.

In acid immersions consisting of acetic acid and 5% sodium hypochlorite, the corrosion behavior was comparable to that of Type 304L steel. The corrosion rates were very low and no true trend in copper addition was observed in the corrosion behavior. All investigated chemistries of Example 2 having a chromium level above 20% were within 1 mm/yr of Type 304L steel.

### EXAMPLE 4

Electrochemical evaluations including corrosion behavior diagrams (CBD) and cyclic polarization studies were performed and compared to the behavior of Type 304L steel.

Corrosion behavior diagrams were collected on the vacuum heat chemistries of Example 2 and commercially

available Type 304L in 3.5% sodium chloride in order to investigate the effects of copper on the anodic dissolution behavior. The anodic nose represents the electrochemical dissolution that takes place at the surface of the material prior to reaching a passive state. As shown in FIG. 4, an addition of at least 0.25% molybdenum and a minimum of approximately 0.40% copper reduce the current density during anodic dissolution to below the measured value for Type 304L steel. It is also noted that the maximum copper addition that allows the anodic current density to remain below that measured for Type 304L steel falls approximately around 0.85%, as shown by the graph of the line identified as Fe21CrXCu0.25Mo in FIG. 4. This shows that a small amount of controlled copper addition while in the presence of 21% Cr and 0.25% molybdenum does slow the anodic dissolution rate in dilute chlorides but there is an optimal amount in order to maintain a rate slower than shown for Type 304L steel.

Cyclic polarization scans were collected on the experimental chemistries of Examples 2 and commercially available Type 304L steel in 3.5% sodium chloride solution. These polarization scans show the anodic behavior of the ferritic stainless steel through active anodic dissolution, a region of passivity, a region of transpassive behavior and the breakdown of passivity. Additionally the reverse of these polarization scans identifies the repassivation potential.

The breakdown potential exhibited in the above mentioned cyclic polarization scans was documented as shown in FIG. 5 and FIG. 6, and evaluated to measure the effects of copper additions, if any. The breakdown potential was determined to be the potential at which current begins to consistently flow through the broken passive layer and active pit initiation is taking place.

Much like the anodic dissolution rate, the addition of copper, as shown by the graph of the line identified as Fe21CrXCu0.25Mo in FIGS. 5 and 6, appears to strengthen the passive layer and shows that there is an optimal amount needed to maximize the benefits of copper with respect to pit initiation. The range of maximum passive layer strength was found to be between 0.5-0.75% copper while in the presence of 0.25% molybdenum and 21% Cr. This trend in behavior was confirmed from the CBD collected during the study of anodic dissolution discussed above though due to scan rate differences the values are shifted lower.

When evaluating the repassivation behavior of the vacuum melted chemistries of Example 2 it showed that a chromium level of 21% and a small molybdenum addition can maximize the repassivation reaction. The relationship of copper to the repassivation potential appeared to become detrimental as the copper level increased, as shown by the graph of the line identified as Fe21CrXCu0.25Mo in FIG. 7 and FIG. 8. As long as the chromium level was approximately 21% and a small amount of molybdenum was present, the investigated chemistries of Examples 2 were able to achieve a repassivation potential that was higher than Type 304L steel, as shown by FIG. 7 and FIG. 8.

A ferritic stainless steel of the composition set forth below in Table 4 (ID 92, Example 2) was compared to Type 304L steel with the composition set forth in Table 4:

TABLE 4

| Alloy | C     | Cr    | Ni   | Si   | Ti   | Cb(Nb) | Other            |
|-------|-------|-------|------|------|------|--------|------------------|
| ID 92 | 0.016 | 20.84 | 0.25 | 0.36 | 0.15 | 0.20   | 0.74 Cu, 0.25 Mo |
| 304L  | 0.02  | 18.25 | 8.50 | 0.50 | —    | —      | 1.50 Mn          |

The two materials exhibited the following mechanical properties set forth in Table 5 when tested according to ASTM standard tests:

TABLE 5

| Mechanical Properties |                      |                  |                      |                   |
|-----------------------|----------------------|------------------|----------------------|-------------------|
|                       | 0.2% YS<br>ksi (MPa) | UTS<br>ksi (MPa) | % Elongation<br>(2") | Hardness<br>$R_B$ |
| ID 92                 | 54.5 (376)           | 72.0 (496)       | 31                   | 83.5              |
| 304                   | 40.0 (276)           | 90.0 (621)       | 57                   | 81.0              |

The material of Example 2, ID 92 exhibits more electrochemical resistance, higher breakdown potential, and higher repassivation potential than the comparative Type 304L steel, as shown in FIG. 9 and FIG. 10.

It will be understood various modifications may be made to this invention without departing from the spirit and scope of it. Therefore, the limits of this invention should be determined from the appended claims.

What is claimed is:

1. A ferritic stainless steel consisting essentially of: about 0.020 or less percent by weight carbon; about 20.0-23.0 percent by weight chromium; about 0.020 or less percent by weight nitrogen; about 0.40-0.80 percent by weight copper; about 0.20-0.60 percent by weight molybdenum; about 0.10-0.25 percent by weight titanium; about 0.20-0.30 percent by weight columbium, optionally one or more members selected from the group consisting of 0.50 or less percent by weight manganese, 0.030 or less percent by weight phosphorus, 0.30-0.50 percent by weight silicon, and 0.040 or less percent by weight nickel, and the balance consisting of iron and unavoidable impurities. 50
2. The ferritic stainless steel of claim 1 wherein the chromium is present in an amount of about 21.5-22 percent by weight.
3. The ferritic stainless steel of claim 1 wherein the copper is present in an amount of about 0.45-0.75 percent by weight. 55
4. The ferritic stainless steel of claim 1 wherein the molybdenum is present in an amount of about 0.30-0.50 percent by weight.
5. The ferritic stainless steel of claim 1 wherein the titanium is present in an amount of about 0.17-0.25 percent by weight. 60
6. The ferritic stainless steel of claim 1 wherein the chromium is present in an amount of about 21.75 percent by weight.
7. The ferritic stainless steel of claim 1 wherein the copper is present in an amount of about 0.60 percent by weight. 65

8. The ferritic stainless steel of claim 1 wherein the molybdenum is present in an amount of about 0.40 percent by weight.

9. The ferritic stainless steel of claim 1 wherein the titanium is present in an amount of about 0.21 percent by weight.

10. The ferritic stainless steel of claim 1 wherein the columbium is present in an amount of about 0.25 percent by weight.

11. The ferritic stainless steel of claim 1 further consisting essentially of about 0.30-0.50 percent by weight manganese.

12. The ferritic stainless steel of claim 1 further consisting essentially of one or more members selected from the group consisting of 0.40 or less percent by weight manganese, 0.030 or less percent by weight phosphorus, 0.30-0.50 percent by weight silicon, and 0.040 or less percent by weight nickel. 15

13. The ferritic stainless steel of claim 1, wherein the concentrations of chromium and molybdenum satisfy Equation 1:

$$0.5 \leq Cr + 3.3Mo \quad \text{Equation 1:}$$

wherein Cr is the concentration of chromium by percent weight, and Mo is the concentration of molybdenum by percent weight.

14. The ferritic stainless steel of claim 1, wherein the concentrations of copper and molybdenum satisfy Equation 2:

$$0.6 \leq Cu + Mo \leq 1.4 \text{ when } Cu_{max} < 0.80 \quad \text{Equation 2:}$$

wherein Cu is the concentration of copper by percent weight, wherein Mo is the concentration of molybdenum by percent weight, wherein  $Cu_{max}$  is the maximum concentration of copper by percent weight.

15. The ferritic stainless steel of claim 1, wherein the concentration of titanium satisfies Equations 3 and 4:

$$Ti_{max} = 0.0044(N^{-1.027}) \quad \text{Equation 3:}$$

wherein  $Ti_{max}$  is that maximum concentration of titanium by percent weight, wherein N is the concentration of nitrogen by percent weight; and

$$Ti_{min} = 0.0025/N \quad \text{Equation 4:}$$

wherein  $Ti_{min}$  is the minimum concentration of titanium by percent weight, wherein N is the concentration of nitrogen by percent weight.

16. A ferritic stainless steel comprising: about 0.020 or less percent by weight carbon; about 20.0-23.0 percent by weight chromium; about 0.020 or less percent by weight nitrogen; about 0.40-0.80 percent by weight copper; about 0.20-0.60 percent by weight molybdenum; about 0.10-0.25 percent by weight titanium; and about 0.20-0.30 percent by weight columbium, wherein the concentrations of chromium and molybdenum satisfy Equation 1:

$$0.5 \leq Cr + 3.3Mo \quad \text{Equation 1:}$$

wherein Cr is the concentration of chromium by percent weight, and Mo is the concentration of molybdenum by percent weight,

wherein the concentrations of copper and molybdenum satisfy Equation 2:

$$0.6 \leq Cu + Mo \leq 1.4 \text{ when } Cu_{max} < 0.80 \quad \text{Equation 2:}$$

wherein Cu is the concentration of copper by percent weight, wherein Mo is the concentration of molybde-

num by percent weight, wherein  $Cu_{max}$  is the maximum concentration of copper by percent weight, wherein the concentration of titanium satisfies Equations 3 and 4:

$$Ti_{max} = 0.0044(N-1.027)$$

Equation 3: 5

wherein  $Ti_{max}$  is that maximum concentration of titanium by percent weight, wherein N is the concentration of nitrogen by percent weight; and

$$Ti_{min} = 0.0025/N$$

Equation 4: 10

wherein  $Ti_{min}$  is the minimum concentration of titanium by percent weight, wherein N is the concentration of nitrogen by percent weight.

\* \* \* \* \*